

## UNITED STATES PATENT OFFICE

GEORGE A. RICHTER, OF BERLIN, NEW HAMPSHIRE, ASSIGNOR TO BROWN COMPANY,  
OF BERLIN, NEW HAMPSHIRE, A CORPORATION OF MAINE

## CHEMICAL PULPING PROCESS

No Drawing.

Application filed May 29, 1930. Serial No. 457,541.

- This invention relates to a chemical pulping process, and more particularly to one in which sulphites are used as fiber liberating agents.
- 5 In the production of so-called sulphite pulps, it is usual practice to employ as the cooking liquor a sulphurous acid solution of a sulphite in which sulphurous acid is present in amount materially beyond that necessary to form the bisulphite. The sulphurous acid or sulphur dioxide content which is neutralizable when an alkali such as caustic soda is added to the liquor, is sometimes known as "free SO<sub>2</sub>," whereas the sulphur dioxide 10 which is combined in the form of the neutral salt or monosulphite is termed "combined SO<sub>2</sub>." The acid sulphite liquors customarily employed for the production of sulphite pulps, e. g., calcium base liquors, have a relatively low combined SO<sub>2</sub> content and a high free SO<sub>2</sub> content, say, 1% to 2% combined and 5% or more free SO<sub>2</sub>.
- In accordance with the present invention, I depart sharply from the usual sulphite process by using sulphite liquors having a high combined SO<sub>2</sub> content and a relatively low free SO<sub>2</sub> content. In fact, the sulphite liquors which I employ have a free SO<sub>2</sub> content less than one-half of their combined SO<sub>2</sub> content. In order to obtain liquors of this type in which the combined SO<sub>2</sub> exists in solution, it is necessary that the sulphite be one of the alkali metal group,—sodium sulphite being preferable because of its general availability and relatively low cost. The liquor may, however, be one containing magnesium and/or calcium sulphite, in which case some of the sulphite may be in suspension rather than in solution, but as the reaction on the cellulosic material progresses to consume dissolved sulphite, the sulphite in suspension may go into solution. I have found that cooking in such liquors to complete fiber liberation is preferably effected at higher temperatures than those used in the usual sulphite process, for the reasons that not only do such higher temperatures effect fiber liberation in as short a period of time as that required for the usual sulphite process, but further that the yield and quality of pulp 15 do not suffer thereby. For instance, as hereinafter described, cooking may be practised advantageously at temperatures even higher than about 325° F. This is especially true when the free SO<sub>2</sub> content of the liquor is less than 1% and the combined SO<sub>2</sub> content is 5% or greater, as in such case cooking at 335° to 375° F. makes possible the complete pulping of chipped wood in from six to eight hours. Even when the free SO<sub>2</sub> content of 20 the liquor is as high as 1% to 2%, if the combined SO<sub>2</sub> content is, in accordance with my invention, more than double this amount, for instance, 5% or greater, I preferably practise cooking at temperatures as high as 335° F. All this will appear hereinafter in greater detail when I give specific examples of procedure. This is in marked contrast to the "scorching" of the fiber and the low yields 25 of pulp resulting when cooking is effected above temperatures of about 250° to 275° F., in the usual acid sulphite liquors. Evidently a high free SO<sub>2</sub> content relative to combined SO<sub>2</sub> content in a sulphite cooking liquor means that the liquor is highly active in the 30 liberation of fiber from raw cellulosic material,—so much so that the temperature and time of cooking must be carefully controlled.
- The use of sulphate liquors in which the combined SO<sub>2</sub> content preponderates materially over the free SO<sub>2</sub> content as hereinbefore described makes possible the production of pulps having characteristics quite different from those associated with the usual sulphite pulps. Thus, a pulp liberated in accordance with the process of the present invention has notably higher strength and tear resistance than that of the usual sulphite pulp. These superior characteristics are doubtless attributable to the fact that a high 35 free SO<sub>2</sub> content in the liquor causes a hydrolysis and weakening of the cellulose fibers, as well as a more extensive removal of pentosans and ligneous matter from the raw cellulosic material than the liquors of the 40 present invention. The fact is that the product of the process of the present invention is much higher in its content of pentosans and ligneous matter than the usual sulphite pulp; and this matter evidently serves as a binder 45

in papers made from the pulp, so that such papers have higher strength than the usual sulphite pulp. The product produced by my process has a light color like that of the usual sulphite pulp, and even though it is difficultly bleachable to pure whiteness because of its comparatively high ligneous content, it constitutes an excellent raw material for blending with ground-wood pulp in the manufacture of a good quality newsprint. It is also especially serviceable as a raw material in the manufacture of papers of high Mullen strength, for instance, glassine papers, wherein its high pentosan content tends to enhance the transparency of the paper. It may further be used as a raw fiber for refinement into a final product of high alpha cellulose content by a series of suitable chemical treatments, including chlorination, digestion in a liquor of suitable alkalinity in either hot or cold condition, and a final bleaching operation.

While there may be various sulphite cooking liquors falling within the purview of my invention, it is distinctly preferable that the combined  $\text{SO}_2$  content of the liquor be about 4% or greater, and that the free  $\text{SO}_2$  content be about 2% or smaller. The use of liquors having such a high combined  $\text{SO}_2$  content gives rise to a high rate of penetration of chemical into the raw cellulosic material, so that in a comparatively short period of time the raw cellulosic material is uniformly impregnated with the liquor and the end of the cooking operation marks a substantially uniform resolution of the cellulosic material into pulp. The process may be carried out substantially in accordance with the standard sulphite mill practice. That is to say, chipped wood, e. g., spruce, is placed in an acid-resistant digester along with the desired cooking liquor, say, one containing 5% combined  $\text{SO}_2$  in the form of sodium sulphite and 1% free  $\text{SO}_2$ . The digester charge is then confined and is heated to about 300° to 335° F., which temperature is maintained for from six to eight hours, in order to ensure complete fiber liberation. The digester contents are then blown and the pulp separated from the spent liquor, which may be subjected to suitable processing for the recovery and reuse of its valuable sodium constituent, when a sodium base liquor has been employed. The pulp may be washed, screened, and subjected to such further treatments as may be desired. In unbleached condition it has a Mullen strength of about 170 and a tear resistance of about 200, which characteristics are superior to those possessed by the usual unbleached sulphite pulp, which has a Mullen strength of about 120 and a tear resistance of about 150. I present herein a table giving various important characteristics of the new fiber produced as hereinbefore described as compared with those possessed by the usual

commercial unbleached kraft and sulphite pulps:

|                                              | Kraft | Un-bleached sulphite | New fiber | 70 |
|----------------------------------------------|-------|----------------------|-----------|----|
| Beaten to same slowness                      |       |                      |           |    |
| Slowness.....                                | 6.00  | 6.00                 | 6.00      |    |
| Shrinkage on drying sheet.....               | 12.00 | 14.00                | 12.00     | 75 |
| Strength of sheet dried without tension..... | 155   | 120                  | 170       |    |
| Tear.....                                    | 250   | 150                  | 200       |    |
| Pentosans.....                               | 6-7   | 3-3.5                | 7-9       |    |
| Color.....                                   | Brown | Cream                | Cream     |    |
| Lignin.....                                  | 6.0%  | 2-3%                 | 10-15%    |    |
| Yield on cooking.....                        | 50%   | 45%                  | 60-75%    |    |

If the free  $\text{SO}_2$  content of the liquor is reduced from 1% to, say, 1/2%, the cooking temperature necessary for the realization of pulp in from six to eight hours ranges from 335° to 375° F., but if it is increased to, say, 2%, the cooking temperature range for the liberation of pulp in the same length of time is from 300° to 335° F. In other words, the higher the free  $\text{SO}_2$  content of the cooking liquor, the lower the temperature necessary to produce within a given period of time a spruce-wood pulp answering approximately the characteristics of the pulp hereinbefore described. The temperature of cooking may further vary with the types of raw material employed,—hardwoods, for example, generally requiring somewhat lower temperatures than soft woods. In any event, however, cooking is effected in a liquor in which the free  $\text{SO}_2$  content is far subordinate to the combined  $\text{SO}_2$  content, and in which the combined  $\text{SO}_2$  is present in high proportion relative to the combined  $\text{SO}_2$  content of the usual sulphite liquors.

If desired, the cooking liquor may be prepared by forming a solution of sodium sulphite of a strength corresponding to both the combined and free  $\text{SO}_2$  content desired in the liquor and adding sulphuric acid and/or niter cake in amount to produce in situ the desired free  $\text{SO}_2$  content. The preparation of the sodium sulphite may be carried out in an apparatus constructed entirely of wood and iron, which is less expensive than the acid-proof apparatus necessary for the production of an acid sulphite liquor. The sodium sulphite solution may then be treated in an acid-proof tank with the desired amount of sulphuric acid and/or niter cake. Such a procedure, which dispenses with the use of sulphur burner gas, is particularly advantageous when niter cake, which is an inexpensive chemical by-product, is used, since, aside from the function of the sulphuric acid content of the niter cake in reacting with the sodium sulphite to produce sulphurous acid and sodium sulphate, the sodium sulphate content of the niter cake and the sodium sulphate reaction product are active chemicals in the cooking

90

95

100

105

110

115

120

125

130

liquor in the sense that as sodium sulphite is exhausted by reaction on the raw cellulosic material, the sodium sulphate undergoes a metathetical reaction with the free  $\text{SO}_2$  content of the liquor to generate sodium sulphite. The same metathetical reaction takes place when the sodium sulphate is formed by the addition of only sulphuric acid to the sodium sulphite solution or when sodium sulphate is added in prepared condition, i. e., as salt cake, to a liquor containing free as well as combined  $\text{SO}_2$ . The sulphite cooking liquor of the present invention may therefore contain sodium sulphate as well as sodium sulphite and free  $\text{SO}_2$ .

If the temperature of cooking is sufficiently high, say,  $375^\circ$  to  $400^\circ$  F., the fiber liberation or pulping of wood may be accomplished in from six to eight hours in a straight monosulphite liquor, for instance, in a liquor containing 5% sodium sulphite. Such a liquor removes less ligneous matter and pentosans from the wood than a liquor containing free  $\text{SO}_2$ , but because it is on the alkaline rather than on the acid side, it may be used in steel digesters similar to those used in the soda and sulphate processes of fiber liberation.

The specific examples of cooking hereinbefore given, in which the raw cellulosic material is converted into a pulp, may be modified considerably, especially as regards time and temperature conditions, when the cooking operation is merely one of a multiplicity of cooking operations or other treatments designed to liberate pulp from the raw cellulosic material. For instance, when the cooking operation is carried out upon raw wood, such as chipped spruce, for about six hours at  $300^\circ$  F., in a liquor containing 5% combined  $\text{SO}_2$  and  $\frac{1}{2}\%$  free  $\text{SO}_2$ , the cooked product is a mass of softened chips containing from 10% to 15% lignin. The yield of this product is 70% to 75%, based on the dry weight of wood used as a raw material. The product may be subjected to mechanical treatment, as in a beater engine or in a Kollergang, to produce pulp; or it may be subjected to further chemical treatment, for

instance, to cooking in other fiber-liberating liquors which are capable of liberating a pulp of high alpha cellulose content therefrom. Rather than being the first of a series of treatments, a cooking operation in which liquors of the composition hereinbefore described may be performed as an intermediate or final treatment.

I claim:

1. A step which comprises treating a fresh sodium sulphite solution with niter cake to convert only a portion of the monosulphite into bisulphite and thereby to produce a sulphite cooking liquor containing free and combined  $\text{SO}_2$  and sodium sulphite. 75

2. In the production of pulp from cellulosic material, the step which comprises cooking such material in an acid sulphite liquor containing sodium sulphate and in which combined  $\text{SO}_2$  is present greatly in excess of 80 free  $\text{SO}_2$ . 85

3. In the production of pulp from raw cellulosic materials, including wood, the step which comprises cooking such materials at a temperature of not less than about  $325^\circ$  F. 90 in a sulphite liquor whose free  $\text{SO}_2$  content is less than one-half of its combined  $\text{SO}_2$  content.

4. A process of producing pulp from raw cellulosic materials, including wood, which comprises cooking such materials at a temperature of not less than about  $325^\circ$  F. in an acid sulphite liquor whose combined  $\text{SO}_2$  content is not less than 4% and whose free  $\text{SO}_2$  content is less than one-half its combined  $\text{SO}_2$  content. 95 100

5. A process of producing pulp from raw cellulosic materials, including wood, which comprises cooking such materials at a temperature of not less than about  $325^\circ$  F. in a sulphurous acid solution of an alkali metal sulphite of the nature of sodium sulphite, whose combined  $\text{SO}_2$  content is not less than 4% and whose free  $\text{SO}_2$  content is less than one-half of its combined  $\text{SO}_2$  content. 105 110

In testimony whereof I have affixed my signature.

GEORGE A. RICHTER.

115

55

120

60

125

65

130

**CERTIFICATE OF CORRECTION.**

**Patent No. 1,915,953.**

**June 27, 1933.**

**GEORGE A. RICHTER.**

**It is hereby certified that error appears in the printed specification of the above numbered patent requiring correction as follows: Page 1, line 79, for "sulphate" read sulphite; and that the said Letters Patent should be read with this correction therein that the same may conform to the record of the case in the Patent Office.**

**Signed and sealed this 12th day of December, A. D. 1933.**

**F. M. Hopkins**

**(Seal)**

**Acting Commissioner of Patents.**